

R. B. FEHR.

METHOD OF AND APPARATUS FOR GIVING HEAT TREATMENT TO MAGNETIC METALS.

APPLICATION FILED SEPT. 28, 1914.

1,188,430.

Patented June 27, 1916.



Witnesses

Wm. C. Dashiell

E. B. McEachern

Inventor

Roy B. Fehr

By

Robt. H. Read

Attorney

# UNITED STATES PATENT OFFICE.

ROY BENNER FEHR, OF STATE COLLEGE, PENNSYLVANIA.

## METHOD OF AND APPARATUS FOR GIVING HEAT TREATMENT TO MAGNETIC METALS.

1,188,430.

Specification of Letters Patent. Patented June 27, 1916.

Application filed September 28, 1914. Serial No. 863,890.

*To all whom it may concern:*

Be it known that I, Roy B. FEHR, a citizen of the United States, residing at State College, in the county of Center and State 5 of Pennsylvania, have invented new and useful Improvements in Methods of and Apparatus for Giving Heat Treatment to Magnetic Metals, of which the following is a specification.

This invention relates to a method of and apparatus for heat treating metals such as iron and its alloys to improve its physical and chemical structure for commercial uses. Carbon steels such as hold in solid solution 10 iron carbids in the form of austenite, martensite, troostite, osmandite, or pearlite depend for its physical and chemical properties upon the heat treatment given it. When it is cooled from a molten condition its cooling 15 curve has a sharp "jog" known as the recalescent point where heat is given up by molecular changes in the ferrite and carbids as constituents. Conversely, when the steel is heated up reactions again occur in a 20 reverse sense and heat is absorbed; this is known as the decalescent point. The usual treatment consists in heating it through its critical range represented by the two points mentioned and noting by the indications of 25 a pyrometer the temperature, to ascertain when these points are attained. The decalescent and recalescent points do not coincide on account of hysteresis and other causes within from 20 to 50 degrees centigrade, the 30 decalescent point always being the higher, and as the pyrometer occasions an instrumental error by reason of thermal lag and close calibrating scale the exact moment when the steel reaches the critical tempera- 35 ture is exceedingly difficult to determine with certainty. This is accentuated because different instruments are in practice used in the laboratory and in the shop, and their calibration is not uniformly standardized. The 40 higher the temperature above the decalescent point from which the steel cools the larger the size of its grain, and the grain, texture, tensile strength, ductility and other physical and chemical characteristics depend on the 45 accurate location of the critical point. By reason of the difficulty in practice of accurately locating the jogs in the heat curve a liberal allowance is made in excess of the required temperature, to approach as nearly as 50 possible to the known required temperature. Thus the present practice is in reality only

an approximation toward a perfect result, and there is not the certainty desired as to the crystallization or as to the character of the carbids, or as to the allotropic form of 60 the ferrite containing it.

By my invention the results are rendered very definite, as the decalescent point can be quickly and very accurately determined. I determine the proper point for heat treatment by passing a magnetic flux through the iron or steel while heating and locate the jog in the heating curve instantly, when it occurs, on an electrical indicating instrument inductively related to the magnetic 65 lines of force threading the iron or steel. The magnetic critical point is at about 760 C. in steels of 0.30 carbon and for steels having more than 0.3% carbon this critical point decreases slightly but in any case this point 70 marks the boundary of the alpha form of iron. The point can be regarded as the proper one for refining or quenching all the steels that are given heat treatment. This point is coincident with the decalescent point and the 75 molecular change in the iron which marks the jog of the heating curve is undoubtedly the origin of the change in the magnetic curve. The point is the one where pearlite 80 goes into solid solution.

Recent accurate tests of certain kinds of steel show conclusively that differences of a few degrees (10 to 30) may alter the properties of steel greatly. It will be apparent, therefore, that a direct method of accurately 90 determining the critical point when the metal is finally treated is of prime importance. Inasmuch as when magnetic metals are heated to the decalescent point they lose 95 their magnetic conductivity, I utilize this property by creating at will a magnetic flux through the metal while being heated, and open the magnetizing circuit by a switch repeatedly during the heating. The collapse of 100 the field of force on such sudden rupture of the magnetizing current produces a large deflection in a milli-voltmeter inductively related to the magnetic circuit. The voltmeter deflections are of large magnitude and there 105 is no chance of error in observation when the decalescent point is thus electromagnetically determined. When the point is thus accurately found I quench, temper or anneal the metal according to its required commercial use and secure a product of the best and most uniform nature to meet the desired 110 specifications. I thereby can accurately con-

trol the grain, by removing the metal from the furnace at the exact instant necessary.

My invention therefore consists in treating magnetic metals to accurately locate their critical points of heat treatment by creating at will a magnetic flux in the metal while under heating and definitely indicating the point by magnetic agencies. It comprises also apparatus for carrying out 10 the method embodying means for operating an indicating instrument at will during the heat treatment in accordance with the changes in magnetic flux at different temperatures to locate the critical point for 15 heat treatment. Other features of novelty will be hereinafter more fully described and will be definitely indicated in the appended claims.

In the accompanying drawing illustrating 20 the invention, the figure shows diagrammatically an apparatus by which the invention may be practised.

P is a piece of steel or any magnetic metal to be treated. For purposes of illustration 25 this is shown as an ingot; it may, however, have any form desired, as that of a tool, an axle, a plate, a rod, or in fact any form where high grade steel is required. The article is surrounded by a heat chamber, 30 as a furnace, or may be electrically heated in any known way. Electrical control is preferred by reason of its convenient adjustment, but other modes of heating could be employed.

35 As shown the furnace 4 is heated electrically by a heat-refractory high resistance ribbon, such as nichrome which may be embedded in the furnace walls in the usual way or may be wound on a refractory insulating or insulated tube, as indicated. The 40 ribbon heater is wound non-inductively and the consecutive turns distributed to produce uniform temperature conditions in the tube as by graduating the distance between consecutive turns toward the ends. Adjustment of the heat may be controlled in usual ways by a regulating rheostat, as indicated at 5. The magnetizing current may be furnished by a copper wire surrounding the 45 furnace, but the plan shown is more convenient being a coil of wire wound around an iron yoke 6 which terminates at the sides of the furnace, the metal to be treated being placed with firm contact between the 50 jaws of the yoke, any space between its ends being filled with soft iron bridge pieces 7, 7'. An adjustable resistance 13 is inserted in the magnetic circuit by which the strength of the magnetic field may be regulated. An ammeter is included in the 55 magnetizing circuit, as indicated at 8. The current may be derived from any suitable source as indicated by the signs plus and minus at the supply mains. In the circuit 60 is included a reversing switch 9. Thus

while the article is being heated while carrying magnetic flux the reversing switch may be manipulated to break and reverse the magnetizing current, creating a maximum range of variation of the magnetic 70 flux. I have shown a milli-voltmeter 10 connected with a copper coil 11 wound around the magnetic circuit. The circuit includes a control switch 12. In operating, to find the critical point of the heat curve, the exciting current is adjusted by the rheostat 13 until the ammeter reading is of a proper value to produce a flux of suitable density 75 in the magnetic circuit. The switch 12 is then closed and the reversing switch 9 is 80 opened; the momentary large deflection of the milli-voltmeter is then read. This reading is proportional to the change in magnetic flux from, say, plus 14,000 units with the magnetizing current to a "residual" flux 85 of say plus 7,000 units with no magnetizing current. Switch 9 is then closed in the opposite direction, and a reading is obtained corresponding to a change in flux from plus 7,000 to minus 14,000 units. These operations are repeated at regular intervals 90 during the heating process, and thus there may be obtained two sets of observations, one set for breaking the circuit and the other for making the circuit. One set would be 95 sufficient, but the other set gives a reliable check on the work. When the readings in either set suddenly begin to increase or decrease (according to whether the magnetic induction is above or below the "knee" of 100 the saturation curve of steel) I have a positive indication that the metal in the hottest part of the furnace is becoming non-magnetic and ready for heat treatment.

It should be noted that switch 12 in the 105 secondary circuit is only for the purpose of preventing injury to the pointer of the milli-voltmeter, for when switch 9 is opened from its reversed position, the milli-voltmeter pointer would be deflected in the opposite direction, *i. e.* off its scale. It is therefore advisable to use a milli-voltmeter 110 with its zero at the middle of the scale. In this case switch 12 can be omitted.

The repeated observations of the magnetic 115 condition of the steel during the heating are of great importance in order to determine accurately the exact moment when the metal should be removed from the furnace for annealing, tempering, or hardening. It requires a sensible interval of time (several minutes) for all the metal to pass the critical temperatures, because the phenomenon of decalescence itself requires time, and especially because all parts of the furnace 120 are not at the same temperature. Uniformity of heating throughout the mass of metal is of the greatest importance in heat-treatment, for unless the steel has a uniform temperature at the time of annealing 125 130

or quenching, the grain-size, constitution and physical properties will vary in the same piece. This is particularly true of the larger pieces of steel that are heat-treated. If the galvanometer deflections referred to above show only a gradual change it is safe to conclude that the furnace does not heat uniformly and in such case the furnace should be rebuilt with a view toward equalizing its temperature. My point to point method of determining the critical temperature for heat-treating has a decided advantage over previous methods in that it indicates whether or not the steel has been heated uniformly past the critical temperature.

Having thus described my invention what I claim as new and desire to secure by Letters-Patent is:

- 20 1. The method of treating steel consisting in heating it through a varying temperature, causing a magnetic flux to pass through it from a point outside the source of heat, and instantaneously indicating the difference between the total magnetic induction and the residual magnetism.
- 25 2. The method of treating steel consisting in heating it through a varying temperature, causing magnetic flux to pass through it from a source outside the region of heat, taking repeatedly and instantaneously indications of the flux changes when the steel is passing the decalescent point, and then quenching, annealing or tempering.
- 30 3. Apparatus for treating steel comprising

ing means for heating it through the decalescent point, a magnetic circuit extending away from the source of heat, a coil inductively related to the magnetic circuit remote from the source of heat, and a dead beat indicator controlled by the coil for taking repeated instantaneous indications of the magnetic condition while the steel is passing through the decalescent point.

4. Apparatus for heat treating steel comprising means for heating it through the decalescent point, a magnetizing coil around the magnetic circuit external to the source of heat for creating magnetic flux in the magnetic circuit including the steel to be treated, means for varying the magnetizing current, and means for indicating repeatedly and instantaneously the loss of magnetic properties of the steel.

5. Apparatus for heat treating a magnetic metal comprising means for heating it through the decalescent point, means for supplying magnetic flux imposed outside the region of heat, means for interrupting the flux, and means for indicating the difference between the total magnetic induction in the metal and the residual magnetism.

Signed at State College, in the county of Center and State of Pennsylvania, this 26th day of September, A. D. 1914.

ROY BENNER FEHR.

Witnesses:

V. R. JONES,  
JOHN L. NECHNER.